

## UNITED STATES PATENT OFFICE.

FREDERICK M. BECKET, OF NEW YORK, N. Y., ASSIGNOR TO ELECTRO METALURGICAL COMPANY, OF NEW YORK, N. Y., A CORPORATION OF WEST VIRGINIA.

## METAL-TREATING COMPOSITION.

No Drawing.

Application filed May 22, 1922. Serial No. 562,824.

*To all whom it may concern:*

Be it known that I, FREDERICK M. BECKET, a citizen of the United States of America, residing at 565 Park Avenue, New York, in the county of New York and State of New York, have invented certain new and useful Improvements in Metal-Treating Compositions, of which the following is a specification.

- 10 In a patent issued to me on August 15, 1922, No. 1,425,572, I have disclosed and claimed certain novel alloys comprising silicon and zirconium, usually in association with iron, the silicon being in sufficient amount to prevent the formation of zirconium carbide in proportions to interfere materially either with the preparation of the alloy or with its solution in molten steel. In said patent I have also disclosed and 20 claimed a process whereby such alloys may be prepared in the electric furnace by direct reduction of a charge comprising silica, a zirconium ore, a carbonaceous reducing agent and a source of iron.
- 25 My further researches have shown that the value of alloys of the zirconium-silicon type is considerably enhanced by the presence therein of manganese, with or without certain other elements as mentioned below.
- 30 The manganese may substitute a part or all of the iron in alloys of the ferrosilicon-zirconium type. As in the patent mentioned above, the proportion of silicon should be sufficient to prevent the formation 35 of zirconium carbide in interfering quantities when the alloy is prepared by direct carbon reduction in the electric furnace. When the alloy (or the aggregate mentioned below) is prepared by other methods as described hereinafter, the silicon, zirconium and manganese, with or without iron or other metals or additions, may be combined in any proportions which may be desired, according to the particular result to be 45 accomplished.

My researches have also shown that for certain purposes it is desirable to associate silicon, zirconium and manganese (with or without other elements or additions) in proportions which do not readily yield a homogeneous alloy. In such cases I prepare a mixture of the silicon, zirconium and manganese, or of their alloy combinations with each other or with other metals such as

iron, aggregating or bonding such mixture by means of a metal or material which will not interfere with the intended application of the product. As such binding or aggregating medium I prefer to use lead, particularly where the mixture is to be used for the treatment of steels. I may however use other metallic or non-metallic binders, including fluxes, such as borates, boric acid, fusible slags or the like. The preparation of such aggregates is more fully disclosed in my pending application Serial No. 498-447 filed September 3, 1921.

The present invention relates therefore in its preferred embodiment to a novel composition, alloy or aggregate containing as its essential components silicon, zirconium and manganese; and to the treatment of molten steel with the same. Iron is usually present but is not an essential ingredient. Other metals or elements, or non-metallic additions, may be present in any desired proportion; and as hereinafter pointed out the manganese may be partly or wholly substituted by certain other elements, and notably by calcium or boron, which possess in common with manganese the capability of lowering the melting point of silica-zirconia slags.

I have discovered that the presence of manganese enhances to a considerable degree the deoxidizing and scavenging action of the other two essential components above mentioned, and particularly that of zirconium. I ascribe this observed effect more especially to the powerful fluxing action of the basic manganese oxide, formed as a result of the usual oxidation reactions, upon the oxides of silicon and zirconium concurrently produced. The manganese, which is present as an alloyed or incorporated constituent, is capable when oxidized of promoting to a maximum degree the formation of a fusible slag and hence the production of clean steel. This increase in fusibility corresponds, in other words, to the effect of this basic oxide in lowering the melting point of a silica-zirconia slag. Similar effects in varying degree are obtainable by means of the oxidation-products of certain other elements, and particularly calcium and boron: it is within my invention therefore to substitute the manganese in this composition either wholly or partly by such

other elements. Or as noted above, boric oxid may be otherwise introduced into the composition as a bonding material or a component thereof.

- 5 I have also found that by no means the least advantage which the alloy or aggregate of zirconium, silicon and manganese possesses in comparison with a similar composition of matter without manganese lies 10 in the higher recovery of zirconium obtained in the finished steel in the case of the former. My experiments indicate, for instance, that the percentage of 15 recovery of zirconium in the steel when a zirconium-silicon-manganese combination is used may be at least 10 per cent higher than when combinations of zirconium, silicon and iron are used under otherwise similar conditions.
- 20 My preferred method is to produce the zirconium-silicon-manganese composition directly as an alloy by carbon reduction in the electric furnace by means of the procedure described in the patent above mentioned, the 25 charge being appropriately modified.

However, my present invention is not restricted to a composition of matter made in this particular manner. I have, for instance, obtained the desired result by simple fusion 30 of ferromanganese in the desired proportions with an alloy containing zirconium, silicon and iron. Another method of obtaining the same result is by briquetting or aggregating mixtures of ferrosilicon-zirconium 35 and ferromanganese, using lead or other fusible metal, alloy, flux or substance not objectionable in the composition as a bond; or by stirring ferrosilicon-zirconium and ferromanganese, or a mixture of the two, into a 40 bath of molten lead or other appropriate material and allowing the resultant mass to solidify.

The use of lead as an agglomerating or 45 aggregating medium makes possible the production of certain zirconium-silicon-manganese compositions which it is either difficult or impossible to obtain by means of simple fusion, or by direct reduction methods without the introduction of deleterious 50 percentages of carbon.

The relative proportions of zirconium, silicon and manganese in the alloy or aggregate is determined by the desired composition of the finished steel, and particularly by the 55 percentage of zirconium which it is desired to introduce into the steel bath. Since any or all of the three essential elements of the alloy or aggregate are frequently required to be added not only as deoxidizing and 60 scavenging elements, but also as alloying elements, it is at once evident that the preferred relative proportions cannot be arbitrarily limited to any particular range of composition.

I have for instance, made use of an alloy 65 prepared by carbon reduction in the electric furnace and analyzing as follows:

|           | Per cent. |
|-----------|-----------|
| Zirconium | 13.73     |
| Silicon   | 51.72 70  |
| Manganese | 29.08     |
| Carbon    | 0.05      |

The balance principally iron.

Using metallic lead as a bond, I have produced and made use of an aggregate analyzing as follows:

|           | Per cent. |
|-----------|-----------|
| Zirconium | 18.92     |
| Manganese | 25.20     |
| Silicon   | 25.91 80  |
| Lead      | 12.33     |

The balance principally iron.

By melting ferromanganese with an alloy of silicon, iron and zirconium, I have produced such alloys as the following:

|           | No. 1.<br>Per cent. | No. 2.<br>Per cent. |
|-----------|---------------------|---------------------|
| Zirconium | 6.41                | 12.30               |
| Silicon   | 50.54               | 28.92 90            |
| Manganese | 20.05               | 28.36               |
| Iron      | 22.34               | 29.37               |

While it is not my contention that as a rule the manganese content of the alloy or aggregate should be high enough to preclude the use of ordinary ferromanganese as a ladle addition, yet it is possible to produce a combination of zirconium, silicon and manganese of such an analysis as to introduce the necessary amounts of these three elements by a single addition of the above-described alloy or aggregate for any given grade of steel.

In the treatment of steel I prefer to introduce my novel product as a ladle addition, although under exceptional conditions it may be added in the furnace.

The amount of manganese which the alloy or aggregate contains largely influences the cost of manufacture, especially when present above a certain amount. From practical considerations I prefer usually to limit the manganese content to 50% or under.

Where it is desired for any sufficient reason to use a zirconium-silicon-manganese alloy or aggregate for the purpose of introducing in one addition the amounts of these three elements which are desired in the manufacture of ordinary carbon or alloy steels, I have found it advantageous in many instances to employ compositions analyzing as follows:

|           | No. 1.<br>Per cent. | No. 2.<br>Per cent. |
|-----------|---------------------|---------------------|
| Manganese | 50.                 | 40 125              |
| Silicon   | 25.                 | 20                  |
| Zirconium | 3.5                 | 20                  |

The balance principally iron.

While I have emphasized in the foregoing the advantages possessed by my composition containing manganese as compared with similar compositions containing zirconium and silicon but without manganese, I wish to point out that, when the silicon content of my novel product is comparatively low, it is possible to regard it essentially as an improved modification of ferrozirconium, in which the iron content of the latter is largely or in part replaced by manganese. Such compositions I regard as within my present invention.

I have found that the use of a zirconium-silicon-manganese composition as an addition agent to molten steel confers upon the finished product the desirable properties characteristic of zirconium-treated steels, whether the addition is in the form of an alloy or of an aggregate containing lead or other fusible binder; and that these desirable characteristics are obtainable with a minimum percentage of added zirconium, by reason of the relatively high recoveries of this metal in the finished steel.

The use of these alloys or compositions is not limited to the treatment of steel, as they are also applicable to the treatment of molten metallic baths in general, including for example cast iron, bronzes, copper, and other non-ferrous metals and alloys.

Claims:

1. A composition suitable for treating molten metal and comprising as its essential components, zirconium, silicon, and an effective quantity of a non-ferrous component capable of lowering the melting point of zirconia-silica slags, said composition containing zirconium not combined with carbon, and having a silicon percentage in excess of half the zirconium percentage.

2. A composition suitable for treating molten metal and comprising as its essential components, zirconium, silicon, and an effective quantity of manganese, said composition containing zirconium not combined with carbon, and having a silicon percentage in excess of half the zirconium percentage.

3. An alloy comprising as its essential

components, zirconium, silicon, and an effective quantity of manganese, said composition containing zirconium not combined with carbon, and having a silicon percentage in excess of half the zirconium percentage.

4. A composition suitable for treating molten metal and comprising as its essential components, zirconium, silicon and manganese, and a fusible bonding material therefor.

5. A composition suitable for treating molten metal and comprising as its essential components, zirconium, silicon and manganese, and a fusible bonding material therefor, said bonding material comprising lead.

6. Process of treating molten metal comprising introducing thereinto a composition comprising zirconium, silicon, and an effective quantity of manganese, said composition containing zirconium not combined with carbon, and having a silicon percentage in excess of half the zirconium percentage.

7. Process of treating molten metal comprising introducing thereinto a composition comprising zirconium, silicon, manganese and lead.

8. Process of treating molten metal comprising introducing thereinto a composition comprising zirconium, silicon, and an effective quantity of a non-ferrous component capable of lowering the melting point of zirconia-silica slags, said composition containing zirconium not combined with carbon, and having a silicon percentage in excess of half the zirconium percentage.

9. Process of treating molten metal comprising introducing thereinto a composition comprising zirconium, silicon, and an effective quantity of a non-ferrous element yielding oxidation products capable of lowering the melting point of zirconia-silica slags, said composition containing zirconium not combined with carbon, and having a silicon percentage in excess of half the zirconium percentage.

In testimony whereof, I affix my signature.

FREDERICK M. BECKET.